

1

2,780,598

**METAL WORKING AND LIQUID COOLANTS  
THEREFOR**

Thomas H. Cafcas, Chicago, Ill., assignor to Standard Oil Company, Chicago, Ill., a corporation of Indiana

No Drawing. Application March 30, 1954,  
Serial No. 419,905

5 Claims. (Cl. 252—33.2)

This invention relates to metal working and more particularly pertains to improved liquid coolants for use in metal working operations.

In metal working operations, liquid coolants are employed to prevent overheating of the work piece and the tool. The liquid coolant functions also to lubricate the contacting surfaces of the tool and work piece. The various metal working operations which employ liquid coolants are those such as cutting, turning, drilling, grinding, and similar operations performed on metals such as iron, steel, copper, bronze, and the like. In the usual metal working operation, the tool and work piece are washed with the coolant which removes the metal particles formed during the metal working operation and also cools the tool and work piece. Provision is usually made for removing at least a part of the metal particles by settling before recirculating the coolant. If the metal particles are not substantially removed from the coolant prior to recirculation, the metal chips are recirculated to the point of contact of the tool and work piece and seriously interfere in the metal working operation. In a metal grinding operation, for example, if the metal grindings are not substantially removed from the coolant before the latter is recirculated to the point of contact of the grinding wheel with the metal work piece, the pores and cavities of the grinding wheel become filled with the grindings. This condition is commonly called "wheel-loading." In this condition the grinding wheel is less abrasive and has uneven projections on its surface. When grinding with such a wheel, the finished work piece may have a scoured surface, chatter marks, and a non-uniform, roughened finish. The grinding wheel which has its surface loaded with metal grindings will not grind the work piece as rapidly as a fresh wheel since its abrasiveness is reduced, and the operator must necessarily work at a slower rate. As the grinding wheel becomes loaded with metal grindings, it develops grooves on its surface which require the wheel to be dressed to a level or uniform surface. Because dressing of the wheel removes useful abrasive surface, the life of the grinding wheel is greatly reduced. In addition, the dressing operation decreases the time during which the grinding wheel and its operator are available for grinding operations.

An object of this invention is to provide a liquid coolant useful in metal working operations and which has the ability to settle rapidly the metal particles in the coolant solution. Another object of this invention is to improve metal working operations by prolonging tool life, increasing the speed of metal working operation, producing finished work pieces having smoother finished surfaces, and in general to increase the efficiency and effectiveness of metal working operations. Other objects and advantages will be apparent in the course of the detailed description of the invention.

It has been discovered that if a small amount of an alkylene diamine tetraacetic acid, or the ammonium or alkali metal salt thereof, is added to a liquid coolant such as the soluble-oil type or the oil-free aqueous type which

2

is then used in a metal working operation, the metal particles settle more rapidly in the coolant solution. It has also been discovered that these compounds impart rust-proofing properties to the coolant. The alkylene diamine derivative may be a butylene-, propylene-, methylene-, and is preferably an ethylene diamine tetraacetic acid or the ammonium or alkali metal salt thereof. The alkali metal salt, particularly the sodium salt, of ethylene diamine tetraacetic acid is preferred. The mono-, di-, tri-, or tri-sodium salt may be employed. The alkylene diamine tetraacetic acid or its ammonium or alkali metal salt, which shall hereinafter be referred to as the settling agent, may be added in an amount between about 0.05 to 20%, preferably 0.1 to 10%, to a concentrate of the coolant which may be of the soluble-oil type or the oil-free aqueous type. The concentrate may then be diluted with between about 5 to 150 parts of water and used in metal working operations in this diluted form as a coolant of superior metal particle settling ability. The diluted form which is used in metal working operations may contain between about 0.001 to 5%, preferably 0.01 to 0.5% of the metal particle settling agent.

The settling agents of this invention are effective in coolants such as the soluble-oil type and the oil-free aqueous type. The settling agent may be added to the concentrated form or to the diluted form of the coolant as used in the metal working operation. It is more conveniently added to the concentrate form. The soluble-oil type concentrate generally comprises base oil and an oil-in-water emulsifying agent. It usually contains a rust-proofing agent and optionally it may contain varying amounts of dispersing agents, bactericides, and the like. Examples of conventional formulæ for soluble-oils to which the settling agent may be added in amounts of about 0.05 to 20% are illustrated in Formulae A and B which follow. In these formulations and wherever a percentage, part, or portion is expressed in the specification or claims, it is intended on a weight basis which is based upon the total components listed therein.

*Formula A*

|                     | Weight percent |
|---------------------|----------------|
| Base oil            | 45-95          |
| Emulsifying agent   | 2-30           |
| Dispersing agent    | 0-5            |
| Rust-proofing agent | 0-5            |
| Bactericidal agent  | 0-1            |
| Load carrying agent | 0-20           |
| Water               | 0-3            |

*Formula B*

|                     | Weight percent |
|---------------------|----------------|
| Base oil            | 1-20           |
| Emulsifying agent   | 10-30          |
| Rust-proofing agent | 0-5            |
| Dispersing agent    | 0-5            |
| Bactericidal agent  | 0-1            |
| Load carrying agent | 0-20           |
| Water               | 40-90          |

A general formula for concentrates of the oil-free aqueous-type coolant is set forth below in Formula C. The settling agent may be added in an amount between about 0.05 to 20% to the concentrate solution illustrated.

*Formula C*

|                     | Weight percent |
|---------------------|----------------|
| Rust-proofing agent | 5-50           |
| Load carrying agent | 0-20           |
| Dye                 | 0-0.1          |
| Water               | 50-95          |

The soluble oils of Formulae A and B and the oil-free aqueous-type concentrate of Formula C may be diluted with 5 to 150 parts of water and used in the diluted form

as liquid coolants for metal working operations. Examples of other coolants to which the settling agent may be added are disclosed in U. S. P. 2,436,046 of N. E. Lemmon et al.; U. S. P. 2,231,214 of R. F. Nelson et al.; U. S. P. 2,252,385 of G. H. Orozco; and U. S. P. 2,289,536 of W. E. Bradley.

The soluble-oils of Formulae A and B contain varying amounts of a base oil. The base oil comprises a hydrocarbon oil such as petroleum or a synthetic hydrocarbon oil. The base oil should have a Saybolt viscosity of about 60 seconds or more at 100° F. and preferably has a Saybolt viscosity of about 75 to 150 seconds at 100° F. The soluble-oil of Formula A is the type most commonly used by metal working industries and it contains 45 to 95% of base oil, preferably between about 75 to 90%.

Suitable emulsifying agents which may be used in the soluble-oil compositions are oil-in-water emulsifiers such as the soaps of preferentially oil-soluble sulfonic acids, soaps of naphthenic acids, soaps of rosin acids and other emulsifying agents such as the non-ionic emulsifiers. Examples of suitable non-ionic emulsifiers are the ethylene oxide condensation products with sorbitan oleates, laurates, and the like. The soap of the preferentially oil-soluble sulfonic acid, naphthenic acid, rosin acid, or the like, is preferably an ammonium, amine, or alkali metal soap. For example, organic naphthenates such as diethanolamine and triethanolamine naphthenate may be used. The soaps of the preferentially oil-soluble sulfonic acids may be prepared by reacting a petroleum distillate with sulfuric acid and neutralizing the organic sulfonic acids thus produced with an appropriate alkaline solution such as an aqueous solution of sodium hydroxide. Either a single emulsifying agent or a mixture of two or three emulsifying agents may be employed in the soluble-oil. For example, the total emulsifying agent used may be comprised of 5 to 25% of sodium rosinate and 75 to 95% of a sodium sulfonate, and this latter mixture of emulsifying agents is preferred for use in the soluble-oil. In general, the total amount of emulsifying agents may comprise between about 2 to 30%, preferably about 5 to 20% of the soluble-oil.

Any of a wide variety of effective rust-proofing agents may be employed in the soluble-oil. For example, the alkylolamines such as mono-, di-, and triethanolamine, propanolamine, butanolamine, and the like, the hydroxamic acid derivatives such as naphthene hydroxamic acid, the ammonium, amine, or alkali metal chromates, salts such as the ammonium, amine, or alkali metal salts of nitrous acids, e. g. sodium nitrite, and the like, may be used. The emulsifying agents generally have some degree of rust-proofing ability and thus serve a double function in the soluble-oil coolant. The soaps of preferentially oil-soluble sulfonic acids are notable examples of such a dual functioning agent. The rust-proofing agent is usually employed in the soluble-oil in amount between about 0.1 to 5%, preferably about 0.25 to 1%. It has also been noted that if the soluble-oil or aqueous-type coolant is somewhat alkaline, its rust-proofing ability is somewhat improved.

Suitable dispersing or coupling agents may be contained in the soluble-oil composition to improve the clarity and stability of the soluble-oil. The dispersing agent ordinarily may comprise an approximately equal mixture of water and an alcohol such as a monohydric alcohol, polyhydric alcohol, or alcohol ether. Examples of these alcohols include ethanol, propanol, isopropanol, butanol, diethylene glycol, ethylene glycol monobutyl ether, and the like. It is not always essential to employ the dispersing agent, but it is sometimes desirable to do so particularly to improve the stability of the emulsion of oil when dispersed in widely varying amounts of water. When it is employed in the soluble-oil it is contained therein in a concentration between about 0.5 to 5.0%, preferably between about 1 to 2% by weight. If desired, bactericides such as 0.1 to 1%, ordinarily about 0.25%

of a chlorinated phenol such as tetrachlorophenol, trichlorophenol, or the like may be added to the soluble-oil. Load carrying agents such as sulfurized mineral, animal, or vegetable oil, e. g. sulfurized lard oil, may be added to the soluble-oil in an amount between about 0.1 to 20%, preferably about 5 to 12% by weight. I have discovered that thiourea functions as a load carrying agent in coolants of the type described herein, and that it is particularly effective in the oil-free aqueous-type coolants. This latter discovery constitutes the subject matter of my application S. N. 419,906 filed on even date herewith.

The soluble-oil containing the settling agent may be prepared by adding emulsifying agent to the base oil in the desired proportion and maintaining the temperature of the mixture at about 75 to 120° F., preferably about 80 to 110° F., and then adding the dispersing agent, rust-proofing agent, bactericide, and load carrying agent in the amount desired to the mixture. The settling agent is then added, in the desired water if any, to the soluble-oil.

The following soluble-oil compositions are illustrations of this invention and should not be interpreted as limiting the scope thereof:

*Example I*

|                                                       | Weight percent |
|-------------------------------------------------------|----------------|
| Sodium sulfonate                                      | 9.0            |
| Sodium rosinate                                       | 1.0            |
| Triethanolamine                                       | 0.20           |
| Oleic acid                                            | 0.20           |
| 30 Tetrachlorophenol                                  | 0.25           |
| Ethyl alcohol                                         | 1.40           |
| Water                                                 | 1.45           |
| Petroleum oil (80 S. S. U. at 100° F.)                | 85.5           |
| Tetrasodium salt of ethylene diamine tetraacetic acid | 0.50           |

*Example II*

|                                                       | Weight percent |
|-------------------------------------------------------|----------------|
| Sodium sulfonate                                      | 2.0            |
| Tween 85 <sup>(1)</sup>                               | 4.0            |
| Petroleum oil (80 S. S. U. at 100° F.)                | 90             |
| 40 Disodium salt of ethylene diamine tetraacetic acid | 4              |

<sup>(1)</sup> Non-ionic emulsifying agent comprising reaction product of ethylene oxide with sorbitan trioleate.

*Example III*

|                                         | Weight percent |
|-----------------------------------------|----------------|
| Sodium sulfonate                        | 4.6            |
| Sodium chromate                         | 4.6            |
| Tween 20 <sup>(1)</sup>                 | 3.7            |
| Petroleum oil (100 S. S. U. at 100° F.) | 4.5            |
| 50 Water                                | 78.6           |
| Ethylene diamine tetraacetic acid       | 4.0            |

<sup>(1)</sup> Non-ionic emulsifier comprising the reaction product of ethylene oxide with sorbitan monolaurate.

The concentrates of the oil-free aqueous-type coolants shown in Formula C are comprised essentially of water containing a rust-proofing agent soluble therein. Examples of highly water-soluble rust-proofing agents are ammonium or alkali metal nitrites or chromates, or the alkylolamines such as mono-, di-, or triethanolamine, morpholine, and the like. Mixtures of such rust-proofing agents may be employed rather than a single agent. An approximately equal mixture of an alkali metal nitrite, e. g. NaNO<sub>2</sub>, with an alkylolamine such as ethanolamine is preferred for use in this oil-free aqueous-type coolant. Bactericides, dyes, load carrying agents particularly thiourea, and other agents may be present in the concentrated or dilute form of the aqueous-type coolant.

The oil-free aqueous-type coolant may be a concentrate solution in water or it may be a mixture of the various agents containing no added water. If the concentrate is prepared on a water-free basis, a mixture in any proportion of the rust-proofing agent and the metal particle settling agent may be used. Preferably, the ratio of rust-proofing agent to settling agent may vary between about 1:3 to 50:1, usually about 5:1. When the concentrate

is prepared as a solution in water it may comprise between about 5 to 50%, preferably about 10 to 30%, of the rust-proofing agent which preferably consists of about equal portions of alkali metal nitrite and ethanolamine, between about 0.05 to 20% and preferably 0.05 to 10% of the settling agent, with water comprising the remainder. The sodium salt of ethylene diamine tetraacetic acid is the preferred settling agent for use in the aqueous-type coolant. The concentrate solution can be made by adding the components in the desired amounts in any sequence to water which is maintained at a temperature of 60 to 120° F., preferably about 100° F., and stirring until solution is complete.

Examples of concentrates of the oil-free aqueous-type coolants are given below:

*Example IV*

|                                                        | Weight percent |
|--------------------------------------------------------|----------------|
| Sodium nitrite                                         | 10             |
| Ethanolamine                                           | 10             |
| Thiourea                                               | 10             |
| Tetra-sodium salt of ethylene diamine tetraacetic acid | 4              |
| Water                                                  | 66             |

*Example V*

|                                                        | Weight percent |
|--------------------------------------------------------|----------------|
| Sodium chromate                                        | 4.6            |
| Tween 20                                               | 3.7            |
| Tetra-sodium salt of ethylene diamine tetraacetic acid | 4.0            |
| Water                                                  | 87.7           |

The effectiveness of the metal particle settling agents of this invention was demonstrated in a grinding operation designed to give a measurable indication of the rate at which the grindings settle. The test comprised grinding a cast iron work piece and circulating coolant in the usual manner by washing the wheel and work piece, allowing the coolant to drain into a sump containing the coolant and grindings, and then recirculating the coolant to wash and cool the grinding wheel and work piece. The sump was divided into two sections by a vertical baffle which had a weir along its upper horizontal edge for the flow of coolant from compartment 1, which held coolant as it descended from the work piece, into compartment 2 wherein the circulating pump picked up coolant and recirculated it to the work piece and tool. Because coolant is recirculated at a rapid rate, the settling rate of the metal particles is usually not sufficient to counteract the circulating direction and rate of travel of the coolant, and consequently, the metal particles tend to be somewhat below but near the surface of the liquid coolant in the sump as it is being circulated. The metal particles will thus normally pass from compartment 1 into compartment 2 and from there they are frequently circulated along with the coolant to the work piece and grinding wheel with attendant damage thereto. In the experiments performed, the cast iron work piece was ground for approximately two hours with recirculation of the coolant, after which time the grinding was discontinued. The coolant was decanted from the sump and the weight of the metal particles in each compartment was estimated. The weight percentage of metal grindings and other particles in each compartment gives an indication as to the effectiveness of the coolant solution for settling metal particles, viz. the higher the percentage of metal particles in compartment 1, the more rapid is the rate of settling of the metal particles. The effectiveness of the settling agent in the soluble-oil type and the aqueous-type coolants is shown by the data set forth in the following table:

6  
TABLE

| 5  | Coolant                           | Wt. percent Settling Agent in Coolant | Metal Particle Settling       |                               |
|----|-----------------------------------|---------------------------------------|-------------------------------|-------------------------------|
|    |                                   |                                       | Wt. per cent in Compartment 1 | Wt. per cent in Compartment 2 |
| 10 | Example I 1—w./o settling agent   | None                                  | 50                            | 50                            |
|    | Example I 1                       | 0.07                                  | 90                            | 10                            |
| 15 | Example IV 2—w./o. settling agent | None                                  | 50                            | 50                            |
|    | Example IV 2                      | 0.06                                  | 90                            | 10                            |

<sup>1</sup> The soluble-oil composition of Example I which is diluted with 7 parts of water to form the coolant used.

<sup>2</sup> The concentrate solution of Example IV which is diluted with 66 parts of water to form the coolant used.

It will be noted from the data in the above table that the coolants which contained the ethylene diamine tetraacetic acid compound were much more effective for settling the metal particles than the same coolant composition which did not contain the settling agent. Visual inspections of the work piece, the grinding wheel, and apparatus were made. It was noted that when the settling agent was employed in the coolant the grinding wheel had a smooth uniform surface free of loading, the grinding apparatus was free of rust, and the work piece had a smooth rust-free surface devoid of scouring.

Other liquid coolant compositions to which the settling agent is added display a similar, although not necessarily equivalent, improvement in the rate of settling of the metal particles within the coolant solution.

It is apparent that many widely different embodiments of this invention may be made without departing from the spirit and scope thereof, and therefore, it is not to be limited except as indicated in the appended claims.

I claim:

1. An emulsifiable soluble-oil comprising between about 45 to 95% of a hydrocarbon oil, between about 2 to 30% of an alkali metal soap of a preferentially oil-soluble sulfonic acid, and between about 0.05 to 10% of an alkali metal salt of ethylene diamine tetraacetic acid.

2. A liquid coolant which comprises from about 5 to 150 parts of water per part of an emulsifiable soluble-oil comprising between about 45 to 95% of hydrocarbon oil, between about 2 to 30% of an alkali metal soap of a preferentially oil-soluble sulfonic acid, and between about 0.05 to 10% of an alkali metal salt of ethylene diamine tetraacetic acid.

3. An emulsifiable soluble oil comprising between about 45 to 95% of a hydrocarbon oil, between about 2 to 30% of an oil-in-water emulsifying agent, and between about 0.05 to 20% of at least one alkylene diamine compound having the general formula



wherein  $n$  is an integer of from 1 to 4, and X is a monovalent radical selected from the class consisting of hydrogen, alkali metals, and ammonium.

4. The composition of claim 3 wherein the alkylene diamine compound is an alkali metal salt of ethylene diamine tetra-acetic acid.

5. The method of minimizing the quantity of suspended metal particles in a liquid coolant which is recirculated onto the tool and work piece during a metal working operation, which method comprises employing a coolant comprising about 5 to 150 parts of water per part of an emulsifiable oil comprising between about 45 to 95% of hydrocarbon oil, between about 2 to 30% of an oil-in-water emulsifying agent, and between

about 0.05 to 20% of at least one alkylene diamine compound having the general formula



monovalent radical selected from the class consisting of hydrogen, alkali metals, and ammonium.

## References Cited in the file of this patent

## UNITED STATES PATENTS

|   |           |           |       |               |
|---|-----------|-----------|-------|---------------|
| 5 | 2,252,385 | Orozco    | ----- | Aug. 12, 1941 |
|   | 2,552,913 | Waugh     | ----- | May 15, 1951  |
|   | 2,631,978 | Bersworth | ----- | Mar. 17, 1953 |